

Nov. 3, 1970

U. M. CEDNÄS ET AL

3,537,809

SWELLING AGENTS USED IN CONJUNCTION WITH REDUCING  
AGENTS IN PROTEINACEOUS TEXTILE SETTING PROCESS  
Filed Dec. 30, 1964

*De-swollen fiber*

*FIG.3*



*FIG.1*



*Non-swollen fiber*

*FIG.2*

*Swollen fiber*



INVENTORS  
EBBA MARIANNE KARRHOLM  
ULLA MARGARETA CEDNÄS  
BY

*Stourell & Stourell*

1

3,537,809

**SWELLING AGENTS USED IN CONJUNCTION  
WITH REDUCING AGENTS IN PROTEINA-  
CEOUS TEXTILE SETTING PROCESS**

Ulla Margareta Cednäs, Molndal, and Ebba Marianne Kärholm, Gothenburg, Sweden, assignors to Stiftelsen Svensk Textilforskning, a foundation of Sweden

Filed Dec. 30, 1964, Ser. No. 422,311

Claims priority, application Sweden, Jan. 8, 1964,  
183/64

Int. Cl. D06m 3/06, 3/10

U.S. Cl. 8—127.6

2 Claims

**ABSTRACT OF THE DISCLOSURE**

Woolen and related proteinaceous materials are set by swelling the material with a strong solution of hydrogen bond breaking agents such as urea, guanadine and monoethanolamine and reducing agents such as water soluble sulphites and bisulphites in water or water soluble organic solvents or mixtures thereof and thereafter deswelling the materials in water while maintaining the desired shape and dimension thereof. Mechanical treatments may be applied to the materials during the deswelling to obtain the desired shape or surface finish thereof and other solvents than water may be used in the deswelling operation.

The term setting a fabric is to be understood as a process of releasing the internal stresses in the material and thereby to stabilize goods in their desired shape or dimension. According to the invention, a substantially permanent setting of the fabric is obtained. After its setting, the fabric is stable to wetting, and the mechanical properties of the fibers do not change appreciably. The cloth or yarns are set in a desired shape which may be smooth or creased, said shape then being the state of equilibrium of the goods desired to be maintained, since the threads in the fabric are set in their wavy state and the internal stresses are balanced. Fabric which is treated in smooth state according to the invention maintains the smooth state even after weaving. After the treatment, an improvement with respect to dry, and particularly wet wrinkling can be observed.

The method of setting yarn and fabric of wool or material chemically similar in nature according to the invention is generally characterized in that the material (FIG. 1) is treated with chemicals swelling the fibers (FIG. 2) in the material, the said chemicals being in a state of solution, such as an aqueous solution, whereafter the textile material is deswelled. During the deswelling, the fiber dimension (FIG. 3) reverts to the initial phase. The material is treated with chemicals breaking the secondary valences, such as hydrogen bonds, together with reducing agents for breaking cystine bridges, said agents breaking the primary valences, and thereby increasing the weight of the goods by about 40 to 400% whereafter the material is deswelled by rinsing with a solvent, so that bridges are rebuilt in the form of both hydrogen bonds and covalent bonds. The deswelling solution may, in addition, contain chemicals facilitating the bridge building, such as hydrogen donators, which results in a setting resistant to renewed water treatment, for example washing.

In a special embodiment of the invention the textile material, subsequent to its treatment with the swelling chemicals is treated by mechanical means to form, for example, pleats, plaits, embossings, for instance by milling, stretching, folding, mangling, embossing, the said deformations being set during the deswelling step. As a result thereof, for example, a tighter and more compact

2

weave structure, elastic stretchability in the warp and/or wet direction, permanent gloss and permanent patterns are obtained.

The swelling chemicals are preferably urea and reducing agent, for example bisulfite or sulfite in aqueous solution, or in aqueous solution mixed with organic solvent, or guanidine and bisulfite, or sulfite in aqueous solution or in aqueous solution mixed with organic solvent, or monoacetanolaminesulfite in high concentration in aqueous solution or sodium- or ammonium thiocyanate and bisulfite or sulfite in aqueous solution or reducing agent, such as bisulfite, sulfite or thioglycolate, in aqueous solution mixed with organic solvent, the fabric being treated with the swelling solution during all of the swelling time or impregnated with the same from about 40% of goods' weight and above said weight whereafter it is stored before the deswelling is carried out. The wool fabric is subjected to a special treatment with a swelling solution containing 20 to 150 g./l. sodium bisulfite or sulfite in a solvent, or 20 to 200 g./l. bisulfite or sulfite in water in combination with 10 to 400 g./l. urea in solvent, or 10 to 600 g./l. urea in water at a temperature of 0 to 100° C., specially 10 to 100° C. and at a pH of about 3 to 9, a maximum effect being obtained at about pH 7, the treatment 10 preferably being carried out at room temperature when the concentration is 200 to 600 g./l. urea and 20 to 200 g./l. bisulfite or sulfite, and at a temperature of 80 to 100° C. with a concentration of about 100 g./l. urea, the swelling bath preferably having a pH of 3 to 9 15 and containing preferably 20 to 200 g./l. bisulfite or sulfite in combination with 10 to 600 g./l. specially 50 to 500 g./l. guanidine, sodium thiocyanate or ammonium thiocyanate, or containing 50 to 500 g./l. monoethanolaminesulfite and the swelling taking place at 0 to 100° C. 20 The swelling is carried out for 2 seconds to 24 hours, the swelling period being inversely proportional to the temperature for example about 5 seconds at 80 to 100° C., and 2 minutes to 24 hours at room temperature, the solvents which may be used being, for example, ethanol, 25 propanol, isopropylalcohol or dioxan.

The deswelling solutions are preferably water or water mixed with an acid, or water mixed with organic solvent, or water mixed with a reagent increasing cross-bridge rebuilding of the type found in keratine, such as 30 formaldehyde. In this case the deswelling preferably occurs at a temperature of 0 to 100° C. and with water or with water and acid, for example acetic acid having a concentration from 0.5 percent by weight to saturation, or with sulphuric acid having a concentration from 0.5 35 percent by weight to saturation, whereafter the fabric may be rinsed with organic solvents, such as petroleum, trichlorethylene, toluene, glycol or glycerol for driving off the deswelling agents.

According to the invention, the deswelling may also be 40 effected by drying when the swelling agents are volatile, for example at 0 to 100° C. for 5 seconds to 24 hours.

The invention will be described in the following, reference being made to the examples for setting wool-fabrics. In all cases an excellent setting was obtained.

60 The setting effect varies according to the swelling agent, concentration, pH, temperature, swelling bath time and to the rinsing and drying conditions.

The following construction applies to the setting of 65 wool fabrics: Binding: serge, 2/2 twill. Yarn number warp and weft: No. 2/42, twisted 450 r.p.m. Modulus length of warp: 390 $\mu$ , weft: 370 $\mu$ .

**EXAMPLE 1**

70 Wool fabric is impregnated with setting solution of 200 g. sodium bisulfite and NaOH to pH=7, (or 50 g. sodium bisulfite and 50 g. sodium sulfite) and 400 g.

urea per liter water, stored at about 20° C. in rolled or folded state for 1 hour (or for 15 minutes to 5 hours), rinsed in water, the fabric being maintained flat during the first part of the rinsing, and dried.

EXAMPLE 2

Wool fabric is impregnated with setting solution of 15 g. sodium bisulfite and 15 g. sodium sulfite and 500 g. urea per liter water and treated according to Example 1.

EXAMPLE 3

Wool fabric is impregnated with setting solution of 400 g. monoethanolaminesulfite (27% SO<sub>2</sub>) per liter water and treated as in Example 1.

EXAMPLE 4

Unwashed wool fabric is treated in a solution of 100 g. monoethanolaminesulfite per liter water for 15 minutes at ~20° C. and then rinsed in water, during the first part of which the fabric must be flat, and dried.

EXAMPLE 5

Wool fabric is treated for 10 seconds at 100° C. in a setting solution of 100 g. sodium bisulfite and sodium hydroxide to pH 7 and 100 g. urea per liter water, rinsed in water, during the first part of which the fabric must be flat, and dried.

EXAMPLE 6

Wool fabric is treated in setting solution according to Examples 1-5, then rinsed in water containing formaldehyde, during which rinsing the fabric must be kept flat, and dried.

EXAMPLE 7

Wool fabric is swelled according to Examples 1-5, then rinsed in water or water containing formaldehyde, during which rinsing the fabric is embossed by mechanical means.

EXAMPLE 8

Wool fabric is swelled according to Examples 1-5, then rinsed in water or water containing formaldehyde, the fabric during the steps of rinsing and drying being over fed both in longitudinal and transverse direction, or being

over fed in one direction and stretched in transverse direction. In this way stretch fabric is obtained.

We claim:

1. A method of setting yarn and fabric textile material containing or consisting of wool or related proteinaceous fibers comprising swelling the material with a solution in water, methanol, ethanol, propanol or dioxane or a mixture of two or more thereof, containing at least 100 grams per liter of a hydrogen bond breaking agent selected from urea, guanidine and monoethanolamine and at least 20 grams per liter of a water soluble sulfite or bisulfite at a pH of from about 3 to about 9, deswelling the material in water while maintaining the desired shape and dimension thereof and rinsing the de-swelled material with an organic solvent.

2. A method as defined in claim 1 wherein the material is subjected to mechanical shaping during the de-swelling treatment.

References Cited

UNITED STATES PATENTS

|           |         |                |       |           |
|-----------|---------|----------------|-------|-----------|
| 2,806,762 | 9/1957  | Ramirez et al. | ----- | 8—127.5   |
| 2,836,185 | 5/1958  | Hervey         | ----- | 8—127.6   |
| 2,850,351 | 9/1958  | Moore et al.   | ----- | 8—127.6   |
| 2,983,569 | 5/1961  | Charle et al.  | ----- | 8—127.6 X |
| 3,051,544 | 8/1962  | Wolf et al.    | ----- | 8—128     |
| 3,151,439 | 10/1964 | Dusenbury      | ----- | 8—127.6 X |

FOREIGN PATENTS

|         |        |                |
|---------|--------|----------------|
| 443,359 | 2/1936 | Great Britain. |
| 968,534 | 9/1964 | Great Britain. |
| 156,139 | 4/1954 | Australia.     |

OTHER REFERENCES

Speakman et al.: Journal of the Textile Institute, pp. T627-T628, July, 1958.

GEORGE F. LESMES, Primary Examiner

J. CANNON, Assistant Examiner

U.S. CL. X.R.

8—128